

Sept. 24, 1957

F. W. GLASER  
CEMENTED CHROMIUM AND CHROMIUM BORIDE MATERIAL  
AND PRODUCTION THEREOF

2,807,075

Filed June 22, 1953

3 Sheets-Sheet 1



FIG. 2



INVENTOR  
FRANK W. GLASER

BY

Greene, Pinches & Durr  
ATTORNEYS

Sept. 24, 1957

F. W. GLASER  
CEMENTED CHROMIUM AND CHROMIUM BORIDE MATERIAL  
AND PRODUCTION THEREOF

2,807,075

Filed June 22, 1953

3 Sheets-Sheet 2

FIG. 3



FIG. 4



INVENTOR.  
FRANK W. GLASER

BY

Greene, Paulson, & Allen  
ATTORNEYS

Sept. 24, 1957

F. W. GLASER  
CEMENTED CHROMIUM AND CHROMIUM BORIDE MATERIAL  
AND PRODUCTION THEREOF

2,807,075

Filed June 22, 1953

3 Sheets-Sheet 3

FIG. 5.



FIG. 6.



FIG. 7.



BY

Greer, Pinella & Surr  
ATTORNEYS

# United States Patent Office

2,807,075

Patented Sept. 24, 1957

1

2,807,075

## CEMENTED CHROMIUM AND CHROMIUM BORIDE MATERIAL AND PRODUCTION THEREOF

Frank W. Glaser, New York, N. Y., assignor to Borolite Corporation, Pittsburgh, Pa., a corporation of Delaware

Application June 22, 1953, Serial No. 363,972

4 Claims. (Cl. 29—182.5)

This invention relates to chromium containing structural materials or compositions of matter which exhibit high hot strength, high heat shock resistance and high corrosion resistance at elevated temperatures, and to the production of such materials.

Among the objects of the invention are structural materials for use in applications such as critical gas turbine parts and the like, which require a material which exhibits high hot strength, high heat shock resistance and high resistance to corrosion under adverse conditions at which other known materials have only a short life or are otherwise unsatisfactory.

Chromium has long been known as a material which has high corrosion-resistance at high temperatures, this corrosion-resistance being secured by the formation of a corrosion-resistant chromium oxide surface stratum on the chromium surface which is exposed to oxidizing combustion gases at high temperatures. However, chromium has only relatively low creep resistance at high temperatures, and for this reason, chromium cannot be used by itself in applications which require low creep resistance at high temperatures.

The best prior efforts to combine chromium with boron for its low creep resistance at elevated temperatures are described in Cole et al. Patent 2,088,838, the material of this patent having become known as "Colmonoy." This Colmonoy material contains as principal ingredients three chromium borides  $\text{CrB}_2$ ,  $\text{CrB}$  and  $\text{Cr}_3\text{B}_2$ , and the conglomerate of these three chromium borides, as described in the "Colmonoy" patent may also contain in free, compounded or alloyed state, minor further additions of chromium, boron, aluminum and iron.

However, the Colmonoy material of the type described in Cole et al. Patent 2,088,838, has excessive brittleness, and could not be utilized for producing, either by itself or by cementing particles thereof with any of the known cementing additions, a cemented material that would exhibit the required high strength, and that would have the capacity of elastically yielding under a load at elevated temperatures as required in certain gas turbine parts.

One phase of the present invention is based on the discovery that by combining chromium with dichromium boride  $\text{Cr}_2\text{B}$ , which has many desirable characteristics that make it superior to other boron rich chromium boride compounds, to wit,  $\text{CrB}_2$ ,  $\text{CrB}$  and  $\text{Cr}_3\text{B}_2$ , there is obtained a material of high hot strength and corrosion-resistance which is much superior to either  $\text{Cr}_2\text{B}$  or  $\text{Cr}$  when used alone for producing gas turbine buckets, rotors and other high temperature metal parts which present critical corrosion problems. An X-ray study of the crystalline structure of dichromium boride  $\text{Cr}_2\text{B}$  indicates that it has an orthorhombic cell of the following parameters:

$$a=14.70\text{A.}; b=7.34\text{A.}; \text{ and } c=4.29\text{A.}$$

Its specific gravity is 6.2 gram/cc., and it has a micro hardness of Vickers DPH 1433. It has a melting point between about 1650° and 1750° C. The dichromium boride  $\text{Cr}_2\text{B}$  will take about 20% chromium in solid solu-

2

tion. It forms a metal rich phase of a much higher order of ductility than other refractory metal borides.

One phase of the present invention relates to a new structural material which in addition to exhibiting high strength, heat shock resistance and corrosion resistance at elevated temperature, also exhibits a substantial desired degree of ductility, the new material combining the dichromium boride  $\text{Cr}_2\text{B}$  with chromium. By choosing the proportion of the excess chromium, the new dichromium boride-excess-chromium material may be given the desired degree of strength and corrosion resistance as well as the desired degree of ductility at elevated temperatures, depending on the temperature at which it is to be used.

The new dichromium boride-excess-chromium material 15 of the invention may to advantage also contain a proportion of chromium oxide  $\text{Cr}_2\text{O}_3$ . For best results, it should be free of carbon impurities greater than about 0.1%, and of iron impurities greater than 0.1 to 0.15%. (Throughout the specification and claims, all proportions 20 are given in weight, unless otherwise specifically stated.) This new material of the invention may be described as boron-poor or boron-deficient dichromium boride material. For securing the minimum required increase in 25 a minimum of about 0.7% boron, and its boron content should not be higher than about 10%. Tests indicate that the  $\text{Cr}_2\text{B}$  plus  $\text{Cr}$  material has a eutectic composition for 4.8% boron content, the eutectic temperature being about 1500° C. at which the material forms a liquid phase.

30 The dichromium boride material  $\text{Cr}_2\text{B}$  without and with the excess of chromium, may be produced by direct synthesis of chromium and boron having a purity of at least about 95%, but for best results the impurities should not exceed about 2.5%, and preferably said impurities should be only about 0.5% or less. The commercially available electrolytic chromium and commercially available amorphous boron of such purity may be used for producing this material. Instead of amorphous boron, crystalline boron may be used. In producing the 35 dichromium boride with the desired excess of chromium or without it, chromium and boron powders are mixed in proportions corresponding to the stoichiometric proportions of  $\text{Cr}_2\text{B}$  with or without the desired excess of chromium, and the mixed powder ingredients are subjected to 40 a heat treatment in which the small amount of boron powder present combines with the chromium into dichromium boride  $\text{Cr}_2\text{B}$ .

45 Satisfactory results are obtained with mixing the required proportions of the chromium powder and the boron powder which have been comminuted to a particle size of 4 to 5 microns, and thereafter subjecting the powder mixture to a further mixing treatment, as in a ball mill, to effect thorough mixture of the different powders and further comminution of the particle size to about  $\frac{1}{2}$  to 2 microns. Good results are obtained by comminuting the individual powders in a gas vortex type pulverizing mill to a particle size of 4 to 5 microns and subsequently ball-milling the mixture of the two powders for about 54 hours. Tests indicate that prolongation of the mixing 50 by ball-milling beyond about 54 hours, does not result in an improved final material.

The ball-milled mixture of the properly proportioned powder ingredients is then heated in a protective atmosphere within a crucible at a temperature of 1300 to 1350° C., or in general between 1200-1500° C. until the amorphous boron has been purified and the reaction between the chromium and boron has reached equilibrium condition. Good results are obtained with a heat treatment of from one to two hours which yields the body of dichromium boride  $\text{Cr}_2\text{B}$  with or without the desired excess of chromium, depending on the proportions of the powder ingredients in the starting powder mixture. The

amorphous boron contains magnesium oxide as a major impurity ingredient, and the heat treatment at 1300° C. in a hydrogen atmosphere within a graphite crucible reduces the magnesium oxide to magnesium, and the resulting magnesium volatilizes at 1300° C., leaving in the crucible the purified boron which forms the desired Cr<sub>2</sub>B as the equilibrium conditions are reached in the progress of the heat treatment.

In an alternative procedure, the dichromium boride Cr<sub>2</sub>B with or without the desired excess of chromium may be obtained by mixing electrolytic chromium and purified boron in the desired final proportions, in which case the initial comminution of the individual powders by a gaseous vortex pulverizing mill is not required. This procedure requires boron of the highest possible purity, of not less than about 95% of its total as chemically analyzed. The properly proportioned mixture of the electrolytic chromium and pure boron powder ingredients is then ball-milled to mix, and then subjected to a similar heat treatment in a graphite crucible within a hydrogen atmosphere at 1300° C. to 1350° C. until the reaction between the chromium and the boron present in the mixture yields at equilibrium condition the dichromium boride Cr<sub>2</sub>B, with or without the desired excess of chromium.

By keeping the boron content of the powder mixture to at most 10%, the resulting material will be free of the boron richer chromium borides, to-wit, CrB, CrB<sub>2</sub> and Cr<sub>3</sub>B<sub>2</sub>.

The carbon impurities of the powder mixture used in making the material of the invention should be kept not larger than 0.1%. Iron impurities of about 0.1 to 0.15% that are introduced by ball-milling with steel balls, are not harmful, but may be eliminated by leaching with HCl.

Shaped articles of high strength, creep resistance, heat-shock resistance, and resistance to corrosion, at elevated temperatures, and having also desired ductility at such temperatures, may be produced out of powder particles of dichromium boride Cr<sub>2</sub>B and excess chromium, by powder metallurgy techniques or ceramic techniques, including hot-pressing as well as cold-pressing or hydrostatic pressing of the desired shapes, followed by sintering. The hot-pressing and the sintering of compacted bodies should be carried out at temperatures between about 1350° and 1500° C. Where the boron content of the combined body is in excess of 4%, the heat treatment and sintering temperature may be increased up to 1700° C. Good results are obtained by hot-pressing and sintering of the compacted powder bodies in an oxidizing atmosphere, such as air, or in an inert atmosphere such as helium or argon or in vacuum. Nitrogen atmospheres should not be used in producing cemented bodies of the invention. It is also detrimental to carry on the hot-pressing or sintering treatments of cemented bodies of the invention in a carbonaceous and/or hydrogen atmosphere, since carbon and hydrogen will have a tendency to reduce chromium oxides which are desirable in the final product. If a carbonaceous and/or hydrogen atmosphere is employed, embrittlement and lowering of the physical properties of the resulting cemented bodies will take place.

In general, satisfactory cemented bodies may be produced by hot-pressing at temperatures of 1400 to 1900° C. or, in general, between 1000 and 2000° C. with pressures of 1/2 to 1 1/2 t. s. i. (tons per square inch). When making bodies by compacting and sintering procedures, good results are obtained by compacting the powder mixture with a pressure of 2 to 4 t. s. i. and subsequently sintering the compact at temperatures above about 1350° C. and close to the melting point of chromium metal. According to available data, pure chromium melts at about 1800° C. ± 20° C.

When producing cemented bodies by hot-pressing, it is desirable to make the hot-pressing die of a material

which does not produce within the die cavity a carbonaceous atmosphere. Dies of zirconium diboride ZrB<sub>2</sub> bonded with 2 to 7% excess boron containing 4 to 33 atomic percent carbon in solid solution or of silicon carbide bonded by silicon nitride, are suitable, in which case the hot-pressing may be done with pressures up to about 10 to 12 t. s. i. If a graphite die is used, the die cavity should be coated with a refractory cement such as zirconium oxide cement, titanium oxide cement, or like cements which are free of or very poor in carbon at the hot-pressing temperature.

The physical characteristics of cemented bodies of the invention will now be described by a series of curve diagrams obtained with cemented bodies containing Cr<sub>2</sub>B+Cr obtained by synthesis, of chromium with amorphous boron in the manner described hereinabove. Similar bodies made with pure crystalline boron have generally similar characteristics, although they vary in some respects.

Figs. 1-7 of the drawings are graphs showing the performance of the various compositions of Cr<sub>2</sub>B and chromium.

Fig. 1 is a curve diagram wherein graph 11 indicates the density of a cemented body formed of Cr<sub>2</sub>B plus Cr for different proportions of Cr<sub>2</sub>B as it increases from zero to 100%. It will be noted that the increase of the Cr<sub>2</sub>B content decreases the density of the material.

Fig. 2 is a curve diagram wherein graph lines 12, 13 show the transverse rupture strength for cemented material Cr<sub>2</sub>B+Cr at 1000° C. for different contents of Cr<sub>2</sub>B as it increases from zero to 100%. This graph shows that the transverse rupture strength is at maximum for a body containing about 35% dichromium boride Cr<sub>2</sub>B. Difficulties have been encountered with bodies having a Cr<sub>2</sub>B content of more than 50% because such bodies have considerably lower ductility than bodies with a smaller Cr<sub>2</sub>B content.

Fig. 3 is a curve diagram wherein graph 5 shows the average Rockwell A hardness for bodies formed of Cr<sub>2</sub>B plus Cr, for different proportions of Cr<sub>2</sub>B as it increases from zero to 100%. It shows that maximum hardness is obtained with a body containing about 80% Cr<sub>2</sub>B.

Fig. 4 is a curve diagram wherein graph 16 shows the electrical resistivity of a cemented body formed of Cr<sub>2</sub>B+Cr, for different proportions of Cr<sub>2</sub>B as it increases from zero to 100%. As shown by the graph, the electrical resistivity increases linearly for bodies wherein the Cr<sub>2</sub>B content increases above 10%, but there is a change in the slope of the graph between zero and 10% increase of Cr<sub>2</sub>B. A study has shown that chromium will take approximately .9 to 1% by weight of boron in solution and this fact may explain the break in this graph at 10% Cr<sub>2</sub>B content, representing a composition containing about .95% boron.

Fig. 5 shows graphs of the oxidation resistance in air and in combustion atmospheres of three bodies of different Cr<sub>2</sub>B content as a function of time. Graph 17-1 indicates the oxidation resistance for a body containing 15% Cr<sub>2</sub>B, graph 17-2 for a body containing 30% Cr<sub>2</sub>B, and graph 17-3, for a body containing 40% Cr<sub>2</sub>B, the balance chromium. The graphs of Fig. 5 show that the corrosion resistance of these materials is excellent and that after the first 200 hours, in which a chromium oxide film develops on the exterior of the body, the further weight gain is very small. Even after 1000 hours' exposure to oxidizing conditions, the appearance of all body specimens subjected to the corrosion tests was excellent and they kept their sharp corners and their original transverse rupture strength.

Fig. 6 is a curve diagram wherein curve 18 shows the transverse rupture strength for a body containing 30% Cr<sub>2</sub>B and 70% Cr, as a function of temperature. Curve 18 shows that the material had a transverse rupture strength in excess of 90,000 p. s. i. (pounds per square

inch) in the temperature range between 1200° and 1250° C.

The cemented material of the invention containing Cr<sub>2</sub>B+Cr has also substantial ductility, and materials of the desired ductility are obtained by increasing the excess chromium content provided that it is not more than 90%, as otherwise the creep resistance of the material is impaired. As the boron content of the body increases, the ductility of the body is decreased. The table below shows the loads required to cause observable bending of molybdenum and Stellite #31 in comparison with desirable Cr<sub>2</sub>B+Cr materials of the invention at 1000° and 1100° C.

Table I

| Material                | Temperatures,<br>° C. | Load for<br>observable<br>bend in p. s. i. |
|-------------------------|-----------------------|--------------------------------------------|
| Molybdenum              | 1,000                 | 25,000                                     |
|                         | 1,100                 | 16,500                                     |
| Stellite No. 31         | 1,000                 | 33,000                                     |
|                         | 1,100                 | 19,000                                     |
| Cr <sub>2</sub> B/70 Cr | 1,100                 | 80,000                                     |
| Cr <sub>2</sub> B/60 Cr | 1,100                 | 105,000                                    |

Fig. 7 is a curve diagram wherein graph 19 shows the deflection rate under a transverse load of 40,000 p. s. i. (pounds per square inch) at 1000° C. for bodies of Cr<sub>2</sub>B+Cr, as the Cr<sub>2</sub>B content is increased from zero to about 80%. The best grade of titanium carbide deflected about  $4 \times 10^{-5}$  inches per minute under similar test conditions, corresponding to the performance of the material of the invention containing 15% Cr<sub>2</sub>B/50% Cr.

As explained above, cemented bodies of the invention containing Cr<sub>2</sub>B+Cr, may be produced either by hot-pressing or by compacting and sintering. To obtain materials of high density approximating the theoretical densities, hot-pressing at 1500° C., at which a liquid phase is formed, with subsequent sintering at the same temperature for 30 to 60 minutes, is desirable. With hot-pressed material which had about 90% theoretical density, almost its full density could be achieved by additional sintering of one hour in air at about 1500° C. Further sintering beyond one hour did not appear to affect the physical properties of the material.

According to a further phase of the invention, a desired material of high corrosion resistance may also be obtained by combining the compound Cr<sub>2</sub>B in powder form with silicon. Thus, whereas Cr<sub>2</sub>B by itself, when subjected to oxidation at 1000° C. in air, exhibited after two hours a weight gain of 15 to 25 milligrams per cm.<sup>2</sup>, an addition of 5 to 20% of silicon reduced the weight gain under the same conditions to 0.3 milligram per cm.<sup>2</sup>. The addition of 5 to 20% silicon metal to Cr<sub>2</sub>B may be accomplished either by mechanical mixing of the ingredients or a synthesis of the component elements of the ingredients in the desired proportions and producing cemented bodies in ways similar to those described above in connection with the production of Cr<sub>2</sub>B+Cr. Cemented bodies consisting of Cr<sub>2</sub>B with 5 to 20% silicon have a transverse rupture strength of 75,000 to 90,000 p. s. i. at 1000° C., and about 56,000 to 60,000 p. s. i. at room temperature. Satisfactory material may be made with as much as 50 to 60% silicon.

By way of example, to produce the desired Cr<sub>2</sub>B+Si material, powders of the Cr<sub>2</sub>B—or of Cr and B in propor-

tions corresponding to the desired amount of Cr<sub>2</sub>B—are mixed with the desired proportion of silicon metal of as high purity as commercially available, which has been comminuted to an average particle size of about 2 to 3 microns. The powder mixture is then further mixed by ball-milling until they have been thoroughly mixed. Good results are obtained by mixing through ball-milling for about 50 hours. The powder mixture is then hot-pressed, followed by sintering or cold-pressing followed by sintering, in the manner described above for Cr<sub>2</sub>B+Cr, to produce cemented bodies of Cr<sub>2</sub>B+Si.

By way of example, a body produced by hot-pressing a body containing Cr<sub>2</sub>B and 20% silicon, had the following physical characteristics:

- 15 Density----- 5.1 gram per cc.  
Electrical resistivity----- 60 microhm cm.  
Transverse rupture strength—at  
1000° C.----- Above 100,000 p. s. i.
- 20 This material has in general, properties similar to the material of the invention described above which contained 50% Cr<sub>2</sub>B+50% Cr.
- It will be apparent to those skilled in the art that the novel principles of the invention disclosed herein in connection with specific exemplifications thereof will suggest various other modifications and applications of the same. It is accordingly desired that the present invention shall not be limited to the specific exemplifications shown or described therein.
- 30 I claim:
1. A hard body of high strength consisting of cemented particles containing essentially 15% to 45% of Cr<sub>2</sub>B and 85% to 55% of a substance selected from Cr and Si, said body being substantially free of CrB, CrB<sub>2</sub> and Cr<sub>3</sub>B<sub>2</sub>.
2. A hard body of high strength consisting of cemented particles containing essentially 15% to 45% of Cr<sub>2</sub>B and 85% to 55% of Cr, said body being substantially free of CrB, CrB<sub>2</sub> and Cr<sub>3</sub>B<sub>2</sub>.
3. A hard body of high strength consisting of cemented particles containing essentially 40% to 95% Cr<sub>2</sub>B and 5% to 60% Si, said body being substantially free of CrB, CrB<sub>2</sub> and Cr<sub>3</sub>B<sub>2</sub>.
4. A hard body of high strength consisting of cemented particles containing essentially 95% to 80% Cr<sub>2</sub>B and 5% to 20% Si, said body being substantially free of CrB, CrB<sub>2</sub> and Cr<sub>3</sub>B<sub>2</sub>.

## References Cited in the file of this patent

## UNITED STATES PATENTS

- 2,084,349 Laise ----- June 22, 1937  
2,171,391 Boecker ----- Aug. 29, 1939

## OTHER REFERENCES

55 McPherson et al.: "Chemistry A Textbook for Colleges," pages 709-716, published by Ginn & Company, 1940.

60 Metal Powder Report, vols. 1-2 (1946-48), pages 75 and 76.

Sinderband: "Properties of Chromium Boride and Sintered Chromium Boride," Metals Trans., February 1949, page 201.

65 Glaser: "Contribution to the Metal-Carbon-Boron Systems," Trans. AIME, J. Metals, April 1952, page 391.